

May 24, 1966

R. H. COOPER ET AL

3,252,818

THERMOSETTING COMPOSITION FOR EXOTHERMIC HOT TOPS

Filed May 1, 1963



Exothermic hot top device fabricated from coated aggregate composition comprised of particulated exothermic hot topping compound and containing alkali metal hydrogen sulfate catalyzed sugar polymer resin binder

INVENTORS.

Ronald H. Cooper  
Robert D. Goodenough  
BY Gerald M. Corbett

BY C. Kenneth Bjork  
AGENT

## 1

3,252,818

**THERMOSETTING COMPOSITION FOR EXOTHERMIC HOT TOPS**

Ronald H. Cooper, Clare, and Robert D. Goodenough and Gerald M. Corbett, Midland, Mich., assignors to The Dow Chemical Company, Midland, Mich., a corporation of Delaware

Filed May 1, 1963, Ser. No. 277,231

2 Claims. (Cl. 106—217)

This application is a continuation-in-part of application Serial Number 99,171, filed March 29, 1961, now abandoned.

This invention relates to improved compositions for use in porous refractory structures which will withstand heat at elevated temperatures such as are encountered upon contact with molten metals. More particularly it is concerned with improved compositions utilizing moldable exothermic compounds for the production of risers and hot tops used in the pouring of molten metals such as iron, ferrous alloys and steels into certain mold forms and to a method of fabricating such structures.

Hot tops and risers, as is well known in the art, are devices that often are employed with molds during the pouring of iron and steel to keep the metal molten in the upper portion of the ingot for as long a period of time as possible. These particularly are used in the pouring of killed steels which undergo substantial contraction upon solidification from the molten state. In use, the hot top which is affixed to the top of the mold acts as a feeder supply for the molten metal during its solidification and accompanying contraction in a mold. The resulting shrinkage cavity, or pipe as it is commonly called, thus occurs in the metal held in the hot top or in the upper portion of the ingot and thereby increases the ingot yield. In recent years, the use of exothermic hot topping compounds, as they have come to be known, has replaced for many operations the conventional insulating type refractory materials long used for these purposes.

It is a principal object of the present invention, therefore, to provide compositions for fabrication into exothermic hot tops, risers and the like porous structures which are readily moldable, have a relatively short curing time, yield a non-hygroscopic end product and are quite inexpensive.

It is also an object of the present invention to provide compositions for fabrication into exothermic hot tops and the like porous refractory structures wherein polymerization of the binder is achieved by an acidic agent which does not decompose upon heating at the curing temperatures nor liberates toxic materials at this temperature.

It is an additional object of the present invention to provide compositions which give ready ease of formation of strong and tough exothermic hot tops along with a minimum amount of after-cleaning of the fabricating apparatus.

It is a further object of the present invention to provide compositions for hot tops which, when used in metal pouring, maintain the metal in molten conditions as long as possible and thereby minimize the severity of the piping in the metal formed in the mold.

It is an additional object of the present invention to provide compositions for use in the preparation of fabri-

## 2

cated structures having adequate and substantially uniform porosity thereby assuring efficient flow and escape means for gases from the molten metal.

It is another object of the present invention to provide compositions which readily are blended into homogeneous mixtures for the fabrication of exothermic hot tops and the like refractory structures.

These and other objects and advantages will become apparent from the detailed description presented herein after and by reference to the accompanying figure.

The drawing in the figure shows schematically a unitary exothermic hot top device prepared from a composition of the instant invention.

In accordance with the present invention, the compositions for use in porous exothermic refractory structures which will withstand heat at elevated temperatures comprise a commonly used exothermic filler material such as a mixture of aluminum, oxidizing agents and refractory powders and a binder system built around novel sugar polymers. In the production of hot tops, for example, the filler can comprise from about 75 to about 95 weight percent or more of the composition with the composite binder system making up the balance.

Fillers useful in the present compositions are those particular materials conventionally used in the manufacture of exothermic hot tops and risers for ingot molds and castings. These materials include, for example, mixtures of aluminum, oxidizing agents such as thermally reducible metal oxides (manganese dioxide or iron oxide) and oxygen containing salts and refractory powders. Additionally, metallic halides such as potassium chloride, sodium chloride and the like can be incorporated into the hot topping compound if desired. These latter materials, if added, impart a fluxing action on the aluminum particles and promote good combustion of the exothermic mixture. The filler material will be in particulated form as is commonly used in preparing the exothermic fabrications. Another illustrative example of an exothermic hot topping composition known in the art is described in U.S. Patent No. 2,591,105. The material taught in this patent is a composition formed from an oxidizable metal such as aluminum (30-50 weight percent), metal oxide such as iron oxide or manganese oxide (5-20 weight percent) i.e. in an amount substantially less than required to completely oxidize the aluminum and a fluoride such as an alkali fluoride or alkali aluminum fluoride (1-5 weight percent) to facilitate the start of the reaction upon contact with molten metal and to facilitate maintaining the reaction to completion. Additionally, this illustrative patented composition can contain sodium nitrate (0-10 weight percent), bentonite (0-2 weight percent), core gum (2-7 weight percent) and granulated grog (remainder).

The binder used in the improved compositions of the instant invention is a polymeric composition resulting from the acid polymerization of monosaccharide sugars, preferably by employing alkali metal hydrogen sulfates as the acidic reaction promoter. These monosaccharides, such as glucose and fructose for example, can be blended directly with the filler. However, conveniently the monosaccharides are produced in situ by hydrolysis of readily obtainable inexpensive di- and polysaccharide hexose sugars as are present in cane sugar, beet sugar, molasses and corn sugar. The hydrolysis results in utilizing the same

acidic material as hydrolyzer which subsequently, at moderately elevated curing temperatures, acts to give polymerization of the monosaccharides. In the production of the exothermic hot top and riser fabrications the amount of saccharide to be employed will range from about 3 percent to about 14 percent by weight of the exothermic aggregate filler. Preferably the sugar concentration will range from about 6 to about 10 percent of the aggregate weight.

Use of a binder having a relatively high sugar content is not desirable for those structures which will be subjected to relatively high temperatures during metal pouring because of the problems that may be introduced by undesirable decomposition of the binder.

For example, hot top devices which contain more than 14 percent by weight of polymerized sugars, may fire and smoke excessively, cause intolerable degrees of metal splattering and give carbonization of the ingot. In fact, at such high sugar levels, the hot tops may not even be capable of the primary requisite to hold the hot metal during the pouring of a heat. Also, at the higher sugar concentrations, the cured product displays a tendency to swell.

On the other hand, hot tops and the like structures prepared using relatively small amounts of sugars can result in refractory structures which do not have the requisite strength after curing.

Useful acidic materials for hydrolyzing and polymerizing the sugar saccharides are acidic compounds (i.e., those having a hydrogen ionization constant,  $K_a$ , greater than about  $1 \times 10^{-2}$ ), including both acids and acidic salts that are non-volatile at the elevated curing temperatures, which do not decompose within this range and which do not produce undesirable decomposition of the polymer-forming constituents during the curing stage. Further, the acidic materials will be solids which are molten at the curing temperatures. Particularly useful materials are the alkali metal hydrogen sulfates, e.g., sodium bisulfate ( $\text{NaHSO}_4$ ), potassium bisulfate ( $\text{KHSO}_4$ ) and lithium bisulfate ( $\text{LiHSO}_4$ ). Sodium bisulfate ( $\text{NaHSO}_4$ ) because of its ready availability, low cost and effectiveness as a hydrolyzer and polymerizing agent has been found to be particularly useful in the present polymer resin forming system.

Acid materials for use as hydrolyzers and polymerization promoters should be stable at the curing temperatures employed. Thus, relatively low boiling aqueous solutions of mineral acids such as hydrochloric, dilute nitric, dilute sulfuric, phosphoric, pyrophosphoric, acetic and the like generally are not useful in the present compositions as hydrolyzers and polymerization promoters as they are volatile below the curing temperatures employed. Therefore, they do not remain in contact with the mix components for a sufficiently long period to give the needed hydrolysis of polysaccharides and subsequent acid promoted polymerization of the resulting monosaccharides into the thermoset binder. Likewise, ammonium sulfate, ammonium persulfate, ammonium sulfamate, ammonium acid sulfate, zinc chloride, monoammonium phosphate and the like are not suitable for use in the present process and composition as all of these produce the corresponding volatile acids at the curing temperatures.

The amount of acid material to be used will vary depending upon the total amount and types of saccharide sugars present. Highly satisfactory polymeric binders result wherein the amount of acidic material is from about 1 to about 8 percent of the particulate exothermic hot topping compound filler. Lower amounts of acid polymerization promoter are employed advantageously when monosaccharides are used directly in the composition. Preferably, the amounts of acid will be somewhat less than the amount of sugar used; for example in an exothermic hot top utilizing from about 6 to about 10 percent sucrose correspondingly from about 1.5 to about 4.5 weight per-

cent of  $\text{NaHSO}_4$  is used as hydrolyzing and monosaccharide polymerizing agent.

The actual binder formation is carried out in the presence of water as a fluidizing medium. From about 3 to about 8 weight percent of water (based on total composition weight) is added to the exothermic filler-saccharide-acid mixture. Preferably the amount of water will range from about 5 to about 7 weight percent of the total binder-filler composition. At higher concentrations, much above 9 weight percent, the structures tend to sag while in the green condition. Also, dimensional instability of the resulting hot top results as the product may undergo undesirable swelling accompanied by the formation of surface cracks during the curing operation. At water contents less than indicated, the cured product may be weak and friable.

The water can be satisfactorily added to a dry-blended mixture of filler and binder. Alternatively, an aqueous solution of the sugar-acid material or a solution of the sugar is used instead of first dry-blending the binder components with the aggregate and then tempering with water.

However, very satisfactory hot tops are produced by first dry blending the ingredients and in most applications and operations this technique may be preferred. In preparing the dry-blends, the saccharide and acid binder components can be premixed and the blend then added to the filler. Alternatively all of the dry components can be blended simultaneously.

The dry blend of binder-filler can be used directly as mixed, or, if desired, can be stored prior to use. The dry binder-alkali metal bisulfite mix also can be stored prior to its use in a refractory composition.

In either of the above suggested methods of dry-blending, it is essential to obtain a substantially uniform and thorough dispersion and interblending of all the ingredients.

The curing of formed refractory structures prepared from the instant compositions is achieved by heating the compositions at temperatures from about 350° to about 450° F., and preferably at about 400° F. for a period of from about 5 to about 30 minutes. The time of cure varies directly, both on the temperature of cure and the thickness and/or size of the device being cured. For conventional hot top fabrications the cure time ordinarily will range from about 8 to about 15 minutes.

Curing the fabrications prepared using the present compositions at thermosetting temperatures below that indicated can yield a relatively weak structure as well as cause difficulties in the decomposition of the polymeric binder upon contact with heat from the molten metal or other sources. Thus, such improperly cured hot top devices may evolve considerable quantities of fire and smoke upon contact with the molten metal and may severely carbonize the resultant solidified metal in a manner similar to that seen when excessive amounts of binder are employed.

At curing temperatures higher than that given herein, degradation and some premature burnout of the polymer with subsequent loss in binding strength may be encountered.

Additionally, if desired, small amounts, from about 0.5 to about 2 weight percent refractory type minerals, iron oxides and other similar materials can be incorporated into the mix to give added thermal shock resistance to the cured product. Also, glues, molasses, pitch, cereals, bentonites, silica flour, sea coal and the like when added in similar amounts can act as thixotropic agents to give better green strength to the formed, uncured device. Small amounts from about 0.25 to about 1.0 percent by weight of thermosetting synthetic resins, e.g., phenol-formaldehyde resins, when incorporated into the blend can serve as strength extenders.

To illustrate the utility of the present new and novel compositions, an exothermic hot top was prepared. In

preparing this device, a commercially available exothermic aggregate was coated with about 8 percent (on the weight of the aggregate) of sucrose, about 3 weight percent  $\text{NaHSO}_4$  and the mixture tempered with about 7 weight percent water. The coating was accomplished by adding the dry binder components to the filler and mixing for about 5 minutes. The water then was added and the mixing continued for an additional 5 minutes. The resulting composition, as freshly prepared, was a damp, pliable and flowable mixture of binder coated filler.

This material was pressed by ramming into a unitary

The wet, plastic "green" composition was dropped into a mold cavity of size as set forth above, rammed lightly and the top surface of the resulting formed product trowelled.

5 The specimens were cured at a predetermined temperature for a given period of time after which the compression strength and surface hardness of the product samples were determined.

10 Table I, which follows, summarizes the results of a number of tests run using various mix compositions and process variables.

TABLE I

| Test No.        | Binder Composition <sup>1</sup> (weight percent) |                  |                      | Cure Time (Min.) | Cure Temperature, F. <sup>°</sup> | Minimum Tensile Strength, lbs/sq. in. | Surface <sup>4</sup> Hardness | Remarks                      |
|-----------------|--------------------------------------------------|------------------|----------------------|------------------|-----------------------------------|---------------------------------------|-------------------------------|------------------------------|
|                 | Sucrose                                          | $\text{NaHSO}_4$ | $\text{H}_2\text{O}$ |                  |                                   |                                       |                               |                              |
| 1               | 8.0                                              | 3.0              | 7.0                  | 10               | 400                               | 170                                   | 90-93                         | Very good mix and core.      |
| 2               | 8.0                                              | 4.0              | 7.0                  | 8                | 400                               | 150                                   | 95-97                         | Excellent mix and core.      |
| 3               | 8.0                                              | 2.0              | 7.0                  | 14               | 400                               | 140                                   | 90-92                         | Good mix and core.           |
| 4               | 6.0                                              | 3.0              | 7.0                  | 12               | 400                               | 100                                   | 90-92                         | Fair mix and core.           |
| 5               | 8.0                                              | 3.0              | 8.0                  | 10               | 450                               | 130                                   | 90-95                         | Good mix and core.           |
| 6 <sup>2</sup>  | 8.0                                              | 3.0              | 7.0                  | 10               | 400                               | 150                                   | 85-87                         | Good mix, not as tacky as 5. |
| 7 <sup>2</sup>  | 8.0                                              | 2.0              | 6.0                  | 12               | 400                               | 135                                   | 85-87                         | Good mix and core.           |
| 8 <sup>2</sup>  | 8.0                                              | 2.0              | 6.0                  | 14               | 350                               | 140                                   | 85-87                         | Good mix and fair core.      |
| 9 <sup>2</sup>  | 8.0                                              | 1.0              | 5.0                  | 16               | 350                               | 130                                   | 85-88                         | Good mix and good core.      |
| 10 <sup>2</sup> | 8.0                                              | 4.0              | 7.0                  | 12               | 350                               | 120                                   | 85-87                         | Good mix and fair core.      |
| 11 <sup>2</sup> | 8.0                                              | 3.0              | 7.0                  | 12               | 350                               | 110                                   | 85-87                         | Do.                          |
| 12 <sup>3</sup> | 8.0                                              | 3.0              | 7.0                  | 10               | 400                               | 100                                   | 75-80                         | Good mix.                    |
| 13              | 10.0                                             | 3.0              | 7.0                  | 12               | 400                               | 125                                   | 90-92                         | Do.                          |
| 14              | 10.0                                             | 2.3              | 8.0                  | 15               | 400                               | 120                                   | 85-87                         | 80-85                        |
| 15              | 39% sodium silicate (control sample)             |                  |                      |                  |                                   |                                       |                               |                              |

<sup>1</sup> Based on weight of aggregate.

<sup>2</sup> Commercial dried corn syrup was used in place of sucrose.

<sup>3</sup> Refined dextrose, or corn sugar, was used.

<sup>4</sup> As determined using a Dietert A.F.S. approved hardness Tester.

hot top mold form under a pressure of about 80 pounds per square inch. The resulting satisfactory green hot top was cured to hydrolyze and to polymerize the binder components at a temperature of about 400° F. for about 10 minutes. After this time, the thermoset hot top in the form of a strong rigid shape was removed from the curing oven.

40 The cured exothermic hot top was then employed in conjunction with an ingot mold during the pouring of hot top steel ingots. The heat from the molten steel being poured decomposed and burned out the cured polymeric sugar based resin and left a strong and uniformly porous refractory structure which provided an easy escape for the gases evolved from the molten metal. The structure, after burnout of the binder, still was strong enough to withstand the ferrostatic head developed by the charge of molten metal.

45 After the ingot had been poured and solidified, the hot top was readily broken away and stripped from the ingot. Substantially none of the burned out structure adhered to the solidified metal.

In a similar manner, sectionalized hot tops and risers also can be fabricated.

50 The following example will serve to further illustrate the present invention but is not meant to limit it thereto.

#### Example

55 Test blocks, 5 x 5 x 2 1/8 inches, were prepared using a commercial exothermic hot topping compound as filler. The aggregate was dry blended with sugar-sodium acid sulfate binder components and the resulting blend tempered with water. The coating of the aggregate by the binder was carried out by mechanically mixing the ingredients in a mix-muller for about 5 minutes.

The sodium acid sulfate was ground, using a micro-pulverizer and passed through an 0.027 inch screen. The sucrose was a commercial product and ground through a micro-pulverizer mill before incorporation into the blend.

55 In a manner similar to that described for the foregoing example, exothermic risers, unitary hot tops and sectional hot tops and the like can be prepared using any of the following as a binder system; glucose-potassium hydrogen sulfate, raffinose-sodium bisulfate, beet sugar-potassium bisulfate, maltose-lithium hydrogen sulfate, fructose-potassium hydrogen sulfate, sucrose-sodium hydrogen sulfate and the like. The binder-filler mix concentrations and techniques to be used with these compositions are to be those as set forth hereinbefore.

60 It is understood that any of the useful saccharide sugars can be satisfactorily polymerized by any of the listed acidic materials.

Various modifications can be made in the present invention without departing from the spirit or scope thereof for it is understood that we limit ourselves only as defined in the appended claims.

We claim:

1. In a thermosetting composition for the fabrication of exothermic hot tops characterized in being thermosetting when heated to a temperature between about 350 and about 450° F. and consisting essentially of a particulated exothermic hot topping compound aggregate filler and a binder the improvement which comprises a binder as based on the filler weight of from about 6 to about 10 percent of a hexose saccharide selected from the group consisting of hexose monosaccharides and acid hydrolyzable polysaccharides and from about 1.5 to about 4.5 percent of an alkali metal acid sulfate selected from the group consisting of sodium hydrogen sulfate, potassium hydrogen sulfate and lithium hydrogen sulfate, and, from about 4 to about 8 percent water, the water weight being based on the total weight of said filler-binder.

2. In a thermosetting composition for the fabrication of exothermic hot tops characterized in being thermosetting when heated to a temperature between about 350 and about 450° F. and consisting essentially of a particulated exothermic hot topping aggregate filler and a binder, the improvement which comprises a binder based 70 on the weight of said aggregate of about 8 percent sucrose,

about 3 percent sodium hydrogen sulfate and about 7 percent by weight water.

2,996,759 8/1961 Smith \_\_\_\_\_ 264—109  
3,021,566 2/1962 Sommer \_\_\_\_\_ 264—109

## References Cited by the Examiner

## FOREIGN PATENTS

## UNITED STATES PATENTS

5 785,984 11/1957 Great Britain.

2,328,644 9/1943 Happe \_\_\_\_\_ 106—40  
2,765,153 10/1956 Gielow et al. \_\_\_\_\_  
2,798,818 7/1957 Pletsch et al. \_\_\_\_\_ 22—147  
2,826,505 3/1958 Jones \_\_\_\_\_ 106—40  
2,875,073 2/1959 Gogek \_\_\_\_\_ 106—38.4 10 P. E. ANDERSON, D. J. ARNOLD, Assistant Examiners.

ALEXANDER H. BRODMERKEL, Primary Examiner.  
ALFRED L. LEAVITT, Examiner.